

## UNITED STATES PATENT OFFICE

PERCY A. E. ARMSTRONG, OF LOUDONVILLE, AND RALPH P. DE VRIES, OF NEWTONVILLE, NEW YORK, ASSIGNEES, BY DIRECT AND MESNE ASSIGNMENTS, TO LUDLUM STEEL COMPANY, OF WATERVLIET, NEW YORK, A CORPORATION OF NEW JERSEY.

## ALLOY STEEL OF HIGH-SURFACE STABILITY AND ARTICLES MADE THEREFROM.

No Drawing. Continuation of application filed January 10, 1921, Serial No. 436,335. This application filed January 14, 1921. Serial No. 437,353.

To all whom it may concern:

Be it known that we, PERCY A. E. ARMSTRONG, a subject of the King of Great Britain, and a resident of Loudonville, county of Albany, and State of New York, and RALPH P. DE VRIES, a citizen of the United States, and a resident of Newtonville, county of Albany, and State of New York, have invented a new and useful Alloy Steel of 10 High-Surface Stability and Articles Made Therefrom, of which the following is a specification.

This application is a continuation of our prior application, Serial No. 436,335, filed 15 January 10th, 1921, and having the same title.

Our invention relates to an alloy steel containing iron, carbon, chromium, silicon and nickel in proportions as stated below; 20 and having high surface stability, that is to say, a high degree of resistance to staining, corroding, oxidizing, and the like agents. The invention also relates to articles made from such alloy steel of high 25 surface stability, of which an article of cutlery is a good example.

The principal part of the alloy is iron. The carbon is preferably kept low, that is to say, under about .50%, but may be from 30 about .05% to about .60%, according to the hardness required in the tool or other article to be produced.

The chromium of the alloy, which also contains nickel and silicon, is preferably 35 from about 5% to about 9%. Less than 5% chromium, though useful, does not produce material of extremely high surface stability, and above 9% of chromium, nickel is of relatively small importance from the 40 standpoint of surface stability, though substantial proportions of silicon can be used to very good advantage.

With chromium from about 5% to about 45 9%, sufficient nickel and silicon is incorporated to make up a total chromium-nickel-silicon content of about 12% to about 15%.

The proportions of chromium, silicon and

nickel in a number of samples which were found to be highly resistant to oxidation, to the action of nitric acid, and to the staining or tarnishing tendencies of vinegar and fruit acids, are given in the following table:

| Chromium | Silicon  | Nickel   | Total—Cr.—Si.—Ni. | 55 |
|----------|----------|----------|-------------------|----|
| Per cent | Per cent | Per cent | Per cent          |    |
| 6.44     | 4.01     | 1.76     | 12.21             |    |
| 6.56     | 3.85     | 2.80     | 13.21             |    |
| 7.56     | 2.98     | 2.98     | 13.48             |    |
| 6.12     | 4.56     | 2.88     | 13.56             |    |
| 6.64     | 4.46     | 3.40     | 14.50             |    |
| 5.28     | 4.70     | 4.72     | 14.70             | 60 |

From the foregoing and other analyses not given here to avoid undue prolixity, we have found that the nickel should preferably be from a quarter to a half of the combined nickel and silicon content of the alloy, but, if desired, the proportion of nickel may be somewhat greater than this, up to about six-tenths of the silicon and 70 nickel taken together. Also as chromium increases from about 5% to about 9%, the quantity of nickel and silicon taken together in general decreases so as to make up a total of chromium-nickel-silicon of about 75 12% to about 15%. Thus with 5% of chromium the nickel and silicon taken together may be from about 7% to about 10%; and with 9% of chromium, nickel and silicon taken together may be from about 3% to 80 about 6%. A good example of the low chromium material may contain: Chromium about 5%, nickel about 5% and silicon about 5%, or a total of 15% of chromium, nickel and silicon taken together. 85

Alloy steel such as described and containing iron, carbon, chromium, nickel and silicon, to give best stable surface qualities, should be heat treated, as by heating to from about 1750° F. to about 1950° F. 90 preferably about 1900° F., and quenching in oil, water, or other quenching medium. The alloy steel may be drawn to suit the purposes for which the alloy is to be used,

generally a drawing temperature of from about 500° to 800° is preferable. This alloy steel may be mechanically worked, as by forging, rolling, or the like operations, or 5 may be cast and used in the cast condition.

This alloy steel is useful for many purposes where high resistance to oxidation hot or cold, and to the action of corroding, tarnishing or the like agents is of importance. Among such uses, in addition to articles of cutlery or other tools for which such material is particularly well adapted, since it readily takes and holds a good cutting edge and a high polish and is extremely 10 resistant to rust and to tarnish, such as caused in ordinary steels by vinegar, fruit juices and the like, we may mention out of many others, the following: valves for internal combustion engines, blades for gas 20 and steam turbines, electrical heating elements to be run at relatively low temperatures up to about 1400° F., hardware, metal cutting tools for withstanding rapid dulling at moderately high temperatures, say 25 up to about 600° F., etc.

Molybdenum up to about 1% can be incorporated with the alloy, the proportion of molybdenum which can be carried increasing with increase in the chromium content. 30 Molybdenum in cutlery blade material produces increased hardness, and the preferable proportion of molybdenum, when used, is about .25% to about .50%. The heat treatment is not materially changed by such addition of molybdenum. Various other elements than as enumerated may be incorporated with the new improved alloy steel, as long as same are not detrimental to the 35 high stable surface characteristics. Same should not in general exceed a total of about 5%.

In the production of our improved alloy steel, cheap high-carbon ferro-chromium can be utilized to good advantage, since so 45 little ferro-chromium is required in making up the melt that the use of ferro-chromium having a relatively high carbon is permissible and the carbon in the alloy still be within the desirable low range. The use 50 of ferro-chromium made by silicon reduction may result in still further economy.

It is to be understood that our invention is not to be limited except as pointed out in our claims, and that the examples given 55 are for the purpose of affording an understanding of the invention and not for its limitation.

We claim:

1. Alloy steel of high surface stability 60 containing carbon about .05% to about .60%, chromium about 5% to about 9%, nickel and silicon, the silicon being over 1%, and the silicon and nickel taken together being sufficient to make up a total chromium-nickel-

silicon content of about 12% to about 15%, 65 and the principal portion of the remainder iron.

2. Alloy steel of high surface stability containing carbon about .05% to about .50%, 70 and containing chromium from about 5% to about 9%, and nickel and silicon, the silicon being over 1% and the nickel and silicon taken together being sufficient to make up a total chromium-nickel-silicon content of about 12% to about 15%, the nickel being at least equal to one-quarter of the silicon and nickel taken together, and the principal portion of the remainder iron. 75

3. Alloy steel of high surface stability 80 consisting of iron, carbon about .05% to about .50%, and from about 12% to about 15% of chromium, nickel and silicon taken together, the nickel content being at least one-quarter of the silicon and nickel taken together 85 and the silicon content being over 1%.

4. Alloy steel of high surface stability 90 containing 12-15% of chromium nickel and silicon taken together, with nickel from 2% to 5%, silicon from 2.5% to 5%, and chromium 7.5% to 5%, an appreciable proportion of carbon not to exceed .6%, and the principal part of the remainder iron. 95

5. Alloy steel of high surface stability 100 containing chromium about 5% up to about 9%, and also containing silicon and nickel, the nickel being at least one-quarter of the silicon and nickel taken together, and the nickel and silicon taken together decreasing from about 7% or 10% to about 3% or 6% as the chromium is increased from its lower 100 to its upper limit.

6. Articles of high stable surface character 105 made from the alloy steel of claim 1.

7. Articles of high stable surface character 110 made from the alloy steel of claim 2.

8. Articles of high stable surface character 115 made from the alloy steel of claim 3.

9. Articles of high stable surface character 120 made from the alloy steel of claim 4.

10. Articles of high stable surface character 125 made from the alloy steel of claim 5.

11. Forged, hardened and tempered tools 130 of highly stable surface character made from the alloy steel of claim 1.

12. Forged, hardened and tempered tools 135 of highly stable surface character made from the alloy steel of claim 2.

13. Forged, hardened and tempered tools 140 of highly stable surface character made from the alloy steel of claim 3.

14. Forged, hardened and tempered tools 145 of high stable surface character made from the alloy steel of claim 4.

15. Forged, hardened and tempered tools 150 of highly stable surface character made from the alloy steel of claim 5.

16. Articles of cutlery of highly stable

surface character made from the alloy steel of claim 1.

17. Articles of cutlery of highly stable surface character made from the alloy steel of claim 2.

18. Articles of cutlery of highly stable surface character made from the alloy steel of claim 3.

19. Articles of cutlery of highly stable

surface character made from the alloy steel 10 of claim 4.

20. Articles of cutlery of highly stable surface character made from the alloy steel of claim 5.

In testimony that we claim the foregoing, we have signed our names hereto.

PERCY A. E. ARMSTRONG.

RALPH P. DE VRIES.